

E. J. WATSON.  
Annealing Apparatus.

No. 222,969.

Patented Dec. 23, 1879.



Witnesses.  
Robert Elliott  
Chas G. Page.

Inventor  
Edwin J. Watson  
Gilmor, Smith & Co.,  
Attorneys

# UNITED STATES PATENT OFFICE.

EDWIN J. WATSON, OF WORCESTER, MASSACHUSETTS.

## IMPROVEMENT IN ANNEALING APPARATUS.

Specification forming part of Letters Patent No. **222,969**, dated December 23, 1879; application filed October 25, 1879.

*To all whom it may concern:*

Be it known that I, EDWIN J. WATSON, of Worcester, in the county of Worcester and State of Massachusetts, have invented certain new and useful Improvements in Mechanism for Annealing Wire; and I do hereby declare that the following is a full, clear, and exact description of the construction and operation of the same, reference being had to the annexed drawing, making a part of this specification, and to the letters and figures of reference marked thereon.

Figure 1 of the drawing is a representation of a side elevation of my device, partly broken away to show my improvements.

My invention relates to improvements in mechanism for annealing wire; and it consists of a furnace having an annealing-vat, in which are placed rollers so arranged as to convey the wire passing over them two or more times through the molten mass in the annealing-vat before it enters the cooling-bath, as will be hereinafter fully described, and particularly pointed out in the claim.

Under my invention I pass the wire or strip through a furnace or bath of molten lead one or more times, by running it around rollers placed in the annealing-vat over the heating-furnace. I then pass the wire or strip through a bath of oil or water, which cools the same; and, finally, I pass it through a die or pair of rolls, where it is cold-rolled and reduced to the required size.

It will be readily understood by those skilled in the art that the texture of the metal is much better when cold-rolled than when rolled or drawn while hot.

The object of passing the wire over the rollers and through the molten mass in the annealing-vat two or more times is, that the wire may be thoroughly annealed, and also that the annealing-vat and furnace may occupy less space than if the wire were passed through as has been customary. In the old devices the wire required to be annealed several times

before being reduced, which required considerable time, and the devices took up too great space.

Referring to the drawing, A designates the vat which contains the bath of molten lead or other metal suitable for annealing purposes. This vat is properly fitted in the top of a furnace, B, which is provided with the usual doors C, grate D, ash-pit E, and doors F, opening into the ash-pit.

The rollers G G, around which the wire or strip is passed, are journaled in suitable brackets, and arranged in pairs within the vat or furnace, so that the wire or rod passing between the same will be properly heated or annealed.

H designates the cooling-vat at one end of the furnace A. This vat is supplied with water or oil for the purpose of cooling the wire preparatory to reducing the same, and it has a roller, I, journaled in a suitable bracket, and arranged so as to guide the wire or strip through the cooling-bath.

Adjacent to the cooling vat or tank are dies or rolls K K, for the purpose of reducing the wire or strip while cold.

As herein shown, the rolls are mounted in suitable housings, and the upper roll rendered adjustable by means of adjustable blocks L and screw-bolts M.

What I claim, and desire to secure by Letters Patent, is—

The furnace B, having an annealing-vat, A, in which are rollers G G, arranged in such a manner as to convey the wire passing over them through the mass in the annealing-bath two or more times before entering the cooling-bath, as and for the purpose set forth.

In testimony that I claim the above I have hereunto subscribed my name in the presence of two witnesses.

EDWIN JUDSON WATSON.

Witnesses:

A. S. WATSON,  
HORACE W. WILLSON.